

July 1, 1930.

C. E. OGDEN

1,769,852

METHOD OF PRODUCING RECTIFYING UNITS

Filed June 27, 1927



Fig 2.



Inventor  
Clarence E. Ogden,  
By Arthur D. Oswald,  
Attorney

## UNITED STATES PATENT OFFICE

CLARENCE E. OGDEN, OF CINCINNATI, OHIO, ASSIGNOR TO THE KODEL RADIO CORPORATION, A CORPORATION OF OHIO

## METHOD OF PRODUCING RECTIFYING UNITS

Application filed June 27, 1927. Serial No. 201,662.

The present invention relates to the method of producing rectifying units particularly of the copper oxide type.

In rectifying units of the copper oxide type, the effectiveness of the units is proportional to the thickness of the layer of oxide on the unit, as well as inversely proportional to the internal resistances of the unit.

10 In the construction of such units I have found that by using chlorine as a catalytic agent during the heat treatment of the metallic plate for the formation of the oxide, the formation of such oxide is facilitated and 15 the layer form materially increased. I have also discovered that the length of time involved in cooling the units after the same have been raised to the required temperature is important to the relation of the internal 20 resistance of the units; that is, the more rapidly the unit is cooled after being raised to the required temperature the lower the internal resistance of the unit.

The object of the present invention is, 25 therefore, to derive in the production of rectifying units the benefits from such discoveries.

In the drawings:

Figure 1 is a view illustrating the method 30 of carrying into effect the present invention.

Figure 2 is a sectional view of a rectifying unit constructed in accordance herewith.

The present method of producing rectifying units is particularly adaptable to the new 35 type of copper oxide units which have lately been developed in which the surface of the layer of copper oxide is again reduced to metallic copper after oxidation by quenching the unit in a bath, for instance, of alcohol and water. In the production of such units it is important that the unit be quenched in the bath when it is at a temperature not higher than 1400 degrees Fahrenheit. As the 40 heat treatment of the units requires that they be raised to approximately 1900 degrees Fahrenheit, there must be an interval of partial cooling before the units are quenched and in order to minimize the internal resistance of the units the period of cooling must 45 be reduced as much as practicable.

The present method consists first in introducing chlorine into the electric furnace 1 from a vial or other container 2 during the heat treatment of the metallic plates in such furnace. The chlorine thus introduced acts 55 as a catalytic agent in the formation of the oxide layer or layers on the metallic plates and enhances the production of such oxide so that the layer formed is comparatively thicker and therefore in the completed unit more 60 effective than where such agent is not employed. After the copper or other metallic plates have been raised to the requisite temperature in the furnace, that is, to approximately 1900 degrees Fahrenheit, for the formation of the oxide, they are then removed in the presence of an electric fan or other mechanical cooling means 3, causing rapid radiation and dissipation of the heat of such units until the temperature is reduced to approximately 1400 degrees Fahrenheit, at 65 which temperature they are quenched in a suitable bath solution in the tank 4. As it is not always possible to control the cooling process before immersion in the bath within 70 the desired limits, I have found that it is ordinarily most practicable to cool the units somewhat lower than the immersion temperature of 1400 degrees Fahrenheit then reheat by placing them in a second furnace 5 before 75 quenching them in the bath, said furnace being maintained at the desired temperature of 1400 degrees Fahrenheit.

Having thus fully described my invention, what I claim as new and desire to 80 secure by Letters Patent is:

1. The method of producing a rectifying unit, comprising raising a copper plate to a temperature of approximately 1900 degrees F. in the presence of oxygen and chlorine, 85 then rapidly partially cooling said plate, then quenching same in a bath adapted partially to reduce the oxide to metallic copper.

2. The method of producing a rectifying unit, comprising raising a copper plate to a 90 temperature of approximately 1900 degrees F. in the presence of oxygen, then rapidly partially cooling said plate, then raising the plate to a quenching temperature, then quenching said plate in a bath adapted 95

tially to reduce the oxide to metallic copper.

3. The method of producing a rectifying unit, comprising raising a copper plate to a temperature of approximately 1900 degrees F. in the presence of oxygen and chlorine, then rapidly partially cooling said plate, then raising the plate to a quenching temperature, then quenching said plate in a bath adapted partially to reduce the oxide to metallic copper.

10 4. In the method of producing a rectifying unit, the step of heating a copper plate to a temperature of approximately 1900 degrees F. in the presence of oxygen and chlorine.

15 CLARENCE E. OGDEN.

20

25

30

35

40

45

50

55

60